

1,460,395

Patented July 3, 1923.

BRITISH

A. 11/13/22

8 713

FRENCH

736964

GERMAN

350771

## UNITED STATES PATENT OFFICE.

OTTO VOGEL, OF DUSSELDORF-OBERKASSEL, GERMANY.

P.D.

## PICKLING BATH AND PROCESS FOR PICKLING IRON AND STEEL.

No Drawing.

Application filed August 27, 1921. Serial No. 495,954.

To all whom it may concern:

Be it known that I, OTTO VOGEL, chemist, a citizen of Germany, residing at Wil-  
denbruchstreet 52, Dusseldorf-Oberkassel,  
5 Germany, have invented certain new and  
useful Improvements in Pickling Baths and  
Processes for Pickling Iron and Steel, of  
which the following is a specification.

The present invention refers to a pickling  
10 bath and a process for pickling iron and  
steel, malleable iron, wrought iron, iron  
alloys as nickel-, chromium-, tungsten-, etc.  
steel.

In pickling such iron and iron articles  
15 by means of acids and acid substances dis-  
solving iron oxides in order to give the iron  
a clean or smooth surface the iron and arti-  
cles from it becomes brittle. In order to  
20 prevent this disadvantage the new pickling  
bath contains besides the acids or acid sub-  
stances aromatic compounds having a ring  
nucleus in which several carbon atoms are  
25 united with a nitrogen atom. Suitable com-  
pounds are chinoline derivatives, as coal tar  
chinoline, synthetical chinoline, isochino-  
line, substituted chinoline compounds as  
30 acridine, alphanaphthochinoline, betanaph-  
thochinoline, chinoline yellow, soluble in  
alcohol or water. Also extracts by means  
35 of acids from the fractions containing such  
bases, obtained in the distillation of coal  
tar are suitable. One may also use such  
fractions from the distillation of coal tar  
containing such bases. Also the syntheti-  
40 cally made products may be added to the  
pickling bath. For instance the raw prod-  
uct from the synthetical production of  
chinoline or naphthochinoline or the molten  
mass from the production of chinoline yel-  
low may be immediately used without puri-  
fication. The amounts of the said additions

may be varied. A favourable action may be  
obtained even by small additions or solu-  
tions of low percentage. A suitable pick-  
ling bath consists of mineral acids, as sul-  
phuric or hydrochloric acid, or organic  
45 acids, as acetic acid, or mixtures of mineral  
and organic acids, or solutions of sodium  
bisulphate, or mixtures of sodium bisulphate  
with acids and 1% of chinoline compounds.  
50

The process for pickling consists in that  
one adds the chinoline compounds to the  
pickling bath before or during the pickling  
operation and that one brings the iron or  
iron article to be treated in this bath until  
55 the oxide layer is sufficiently removed. Then  
one takes the iron from the bath, washes it  
with water or bases, as lime hydrate, soda  
lye or such like and water and dries the  
iron.

I claim:—

1. Pickling bath for iron consisting in  
acid substances dissolving iron oxides and  
aromatic compounds having a nucleus in  
which several carbon atoms are united with  
65 a nitrogen atom.

2. Pickling bath for iron consisting in  
acid substances dissolving iron oxides and  
chinoline compounds.

3. The process for pickling iron which  
70 consists in bringing iron into a bath con-  
taining acid substances dissolving iron ox-  
ides and aromatic compounds having a nu-  
cleus in which several carbon atoms are  
united with a nitrogen atom.

4. The process for pickling iron which  
75 consists in bringing iron into a bath contain-  
ing acid substances dissolving iron oxides  
and chinoline compounds.

In testimony whereof I hereunto affix my  
80 signature.

OTTO VOGEL.

Benzyl acridine